

Oct. 11, 1932.

C. D. SMITH

1,882,526

STENCIL

Filed Dec. 23, 1930



FIG. 1.



FIG. 2.



FIG. 3.

INVENTOR

WITNESS:  
Prof. R. Kitchell

Charles D. Smith  
BY  
Bosser & Harding  
ATTORNEYS.

## UNITED STATES PATENT OFFICE

CHARLES D. SMITH, OF SHARON HILL, PENNSYLVANIA, ASSIGNOR TO THE DALLETT COMPANY, OF PHILADELPHIA, PENNSYLVANIA, A CORPORATION OF PENNSYLVANIA

## STENCIL

Application filed December 23, 1930. Serial No. 504,316.

My invention relates to an improvement in stencils such as are used in connection with the sand blasting of letters or figures on stone, wood, glass, etc., etc. My invention more particularly relates to the production of a stencil which may be repeatedly used.

Heretofore in the preparation of a stencil for use in connection with the sand blasting of stone, wood, and the like, it has been customary to cover the surface of the object to be sand blasted with a plastic or fluid material by means, for example, of heat, permitting the material to harden, and cutting out the letters or figure to be sand blasted. When the sand blasting is completed, the stencil material is removed, but the stencil is necessarily destroyed in the process of removal and for a repetition of the letters or figure a new stencil must be cut. Less usually stencils have heretofore been provided comprising material laid on a paper backing and adapted to be adhered to the surface of an object to be stenciled through the rendering of the material adhesive to the object say, for example, by the application of heat to a surface thereof. Such stencils, however, are subjected to destruction on removal after completion of the sand blast.

Further stencils have been provided comprising desirable material capable of resisting sand blast and adapted to be affixed to the surface to be sand blasted through the medium of an adhesive, as glue. Such stencils, while they are not destroyed in removal from the surface, are undesirable since the surface to which the stencil was adhered must be cleaned to remove the glue and where the surface is of a delicate nature, as for example, where coated with paint, removal of the glue is substantially impossible without injury to the surface.

Now, it is the object of my invention to provide a stencil which may be readily adhered to the surface of an object to be sand blasted and which on completion of the sand blasting may be readily removed from the object without injury and in a condition for reuse. The stencil in accordance with my invention may be repeatedly reused.

In accordance with my invention I provide a stencil comprising laminated sheets, one of which is composed of a material capable of being rendered sufficiently adhesive to a surface to be sand blasted as to maintain the stencil in place during the sand blasting and, at the same time, having insufficient adhesion to cause it, or the surface to which it is applied, injury on removal, and of such a character as to leave the surface to which it is applied without the deposit of any adhesive. The shell of the laminated sheets is composed of a material of such a character as to enable the first described sheet to adhere to it and, at the same time, of such a character as to resist the action of the sand blast. The sheet adapted to adhere to the surface to be sand blasted may be relatively thin compared to the thickness of the sheet adapted to resist the action of the sand blast.

Having indicated in a general way the nature and purpose of my invention, I will proceed to a detailed description thereof with particular reference to the accompanying drawing, in which:

Figure 1 is a sectional view showing a surface to be sand blasted with a stencil embodying my invention associated therewith.

Figure 2 is a perspective view of the subject matter of Figure 1.

Fig. 3 is a sectional view of the stencil shown on a larger scale.

In the drawing *a* indicates a surface to be sand blasted, as for example, the surface of a piece of stone, wood, glass or the like. *b* indicates a sheet of material having the capacity for resisting the action of a sand blast, superimposed upon a relatively thinner sheet of material *c*, to which it is adhered and which in turn is capable of being rendered adherent to the surface *a*. *d*, *d* indicates letters cut through the superimposed sheets *b* and *c* and which are adapted to be sand blasted into the surface *a*.

By way of example, the sheet *b* may be formed by a formaldehyde condensation product or synthetic rubber formed, for example, by digesting a mixture of about 25 pounds of glue, 12 pounds of glycerin and 12 pounds of water for a period of about

twenty-four hours, then cooking at a temperature of about 80° C. for about four hours and finally adding formaldehyde for the production of a water-insoluble condensation product. The material so produced is sheeted in any suitable manner, as for example, by casting or by flowing the material on a surface, for the formation of a sheet of desired thickness.

By way of example, the sheet *c*, capable of being rendered adherent to a surface to be sand blasted, and desirably softer than the sheet *b*, may be cast directly on the sheet *b*, a sheet of light weight blotting paper *e* being interposed between the sheets. The sheet *c*, for example, may be formed by casting on the sheet *b* a composition composed of about 25 pounds of glue, 6 pounds of glycerin and 14 pounds of water. When the sheet *c* has hardened, the exposed surface thereof will desirably be dusted over with talcum powder. It will be noted that the sheet *c* when cast on the sheet *b* will adhere thereto and form a unitary structure. Where a sheet of light weight blotting paper is interposed between the sheets, the blotting paper will become saturated with the composition forming the sheet *c* when it is cast and adherence between the sheets will be permitted, since the composition-impregnated fibres of the surface of the blotting paper lying against the surface of the sheet *f* will tenaciously adhere to sheet *f*.

When it is desired to use the stencil formed as indicated, it is only necessary to wet the exposed surface of the sheet *c* to render it sufficiently adhesive to retain the stencil in place after the wetted surface has been pressed upon the surface to be sand blasted. When the stencil is adhered to the surface to be sand blasted, or previously if desired, the letters or figures to be sand blasted are cut out. Since the material of sheet *b* is strongly resistant to the action of the sand blast, the stencil will be found to be little injured by the sand blast and may be readily stripped off, since the adherence of sheet *c* to the surface, while sufficient to maintain the stencil in place, is not such as to cause the stencil to be injured in its removal. Further, the adherence of the sheet *c* to the surface is not such as to leave any of the composition of which the sheet is formed on the surface. In other words, the stencil on removal will leave the surface clean.

The stencil in accordance with my invention may be adhered with equal readiness and efficiency to surfaces of various kinds, as wood, glass, metal, etc., etc. and may be as readily cleanly removed therefrom and may be safely applied to painted surfaces, since the adherence of sheet *c* will not be such as to injure a painted surface on removal. Further, the stencil in accordance with my invention lends itself to the formation of any de-

sired letters or figures, since it may be readily and cleanly cut, the softer sheet *c* being supported by the harder sheet *b*.

It will be understood that I contemplate as within the scope of my invention the use of any desirable material for the formation of the sheet *b* so long as it is resistant to the action of sand blast and the use of any desired material for formation of the sheet *c* so long as it is capable of being rendered sufficiently adherent to form a unitary structure with sheet *b* and to maintain the stencil in place and, at the same time, insufficiently adherent to cause injury to the stencil or to a surface on its removal.

What I claim and desire to protect by Letters Patent is:—

1. A stencil material for abrasive blasting comprising a laminated sheet including an upper sheet composed of abrasive resistant material, a lower sheet adhered to the upper sheet and composed of a material capable of being rendered tacky by the application of water and an intermediate sheet adhered to both the upper and lower sheets.

2. A stencil material for abrasive blasting comprising a laminated sheet including an upper sheet composed of synthetic rubber and a lower sheet composed of a mixture of glue and glycerine.

3. A stencil material for abrasive blasting comprising a laminated sheet including an upper sheet composed of synthetic rubber, a lower sheet composed of a mixture of glue and glycerine and an intermediate sheet composed of blotting paper.

In testimony of which invention, I have hereunto set my hand, at Philadelphia, Pennsylvania, on this 19th day of December, 1930.

CHARLES D. SMITH.

10

11

11

12

12

13